

C. E. ACKER.  
PROCESS OF PRODUCING ALKALI AND ALKALINE EARTH METALS.  
APPLICATION FILED AUG. 5, 1910.

1,116,865.

Patented Nov. 10, 1914.

2 SHEETS-SHEET 1.

Fig. 1.



Fig. 2.



Witnesses:  
George Cheney  
Jack Hadden

Charles E. Acker Inventor  
By his Attorneys  
Rosenbaum & Stockenagle

C. E. ACKER.

PROCESS OF PRODUCING ALKALI AND ALKALINE EARTH METALS.

APPLICATION FILED AUG. 5, 1910.

1,116,865.

Patented Nov. 10, 1914.

2 SHEETS-SHEET 2.

Fig. 3.



Fig. 4.



Witnesses:

*John G. Blaney*  
*Charles P. Heden*

Inventor  
*Charles E. Acker*  
By his Attorney  
*Benjamin Lankford*

# UNITED STATES PATENT OFFICE.

CHARLES E. ACKER, OF OSSINING, NEW YORK, ASSIGNOR TO THE NITROGEN COMPANY, A CORPORATION OF NEW YORK.

## PROCESS OF PRODUCING ALKALI AND ALKALINE-EARTH METALS.

1,116,865.

Specification of Letters Patent. Patented Nov. 10, 1914.

Application filed August 5, 1910. Serial No. 575,819.

To all whom it may concern:

Be it known that I, CHARLES E. ACKER, a citizen of the United States, residing at Ossining, in the county of Westchester and State of New York, have invented certain new and useful Improvements in Processes of Producing Alkali and Alkaline-Earth Metals, of which the following is a full, clear, and exact description.

10 This invention relates to the production of alkali and alkaline-earth metals, and has for its object the provision of a process whereby such metals may be produced more economically and efficiently than heretofore.

15 United States patent to Edgar A. Ashcroft, No. 801,199, dated October 10, 1905, discloses a process for the production of alkali metals; sodium being obtained by electrolyzing fused sodium chlorid over a molten lead cathode, thereby producing an alloy of lead and sodium, such alloy being thereafter employed while still molten as an anode in connection with a secondary electrolyte consisting of fused sodium hydroxid 20 or fused sodium chlorid; the cathode in this latter operation being of iron or nickel and the alkali metal being liberated thereat, subsequently rising to the surface of the secondary electrolyte from whence it may be 25 drawn off.

I have found in practice that the above described process is open to a number of serious objections which have been brought into notice in attempting to use the various 30 substances heretofore proposed for use as secondary electrolytes. While sodium hydroxid, chlorid, bromid or iodid, may on a small scale or in a laboratory be used to effect the production of sodium in the manner above described, such electrolytes, and in fact all others that have thus far been mentioned or proposed for this purpose, fail to measure up to the commercial requirements. In passing a heavy current of 35 electricity from the surface of molten lead-sodium or like alloy through an electrolyte of fused sodium hydroxid at the temperature at which the alloy was made, to wit, 700°-800° C., substantially no sodium will 40 be liberated at the cathode, and but very little will be obtained at all unless the tem-

perature be reduced to approximately 350° C., which imposes an onerous and uneconomical condition. Then, too, if the current be passed from the alloy through an 55 electrolyte composed of any chlorid, bromid, fluorid, iodid, or a mixture thereof, more or less of the heavy metal is liable to be plated out with the sodium unless the current density on the surface of the alloy 60 is quite low or unless the alloy is quite rich in alkali metal; the latter condition involving uneconomical conditions in the primary cell. A weak alloy may result in the deposition of impure alkali metal at the cathode 65 and in low efficiency in the secondary cell; such objectionable features being possible by reason of the fact that the heavy metal in the alloy may combine with the liberated anion to form a stable salt at the temperature 70 of the operation. If, for example, the secondary electrolyte be fused sodium chlorid and the anode be lead-sodium alloy, the anion will be chlorin, and this will combine with avidity with the sodium in the alloy 75 at the surface thereof; but there is the liability, particularly in the case of a weak alloy, that unless the current density be low, combination to a greater or less extent between the lead and chlorin may occur, resulting in the formation of lead chlorid,— 80 a very stable conducting salt, which mixes with the molten sodium chlorid and is then decomposed by the current with deposition of lead at the cathode. This and other objectionable actions are apt to occur not only 85 in connection with the use of lead alloy and a secondary electrolyte of sodium chlorid, but with other alkali or alkaline-earth metal alloys and with numerous salts. The current efficiency in the secondary cell with chlorid electrolytes is always very low because the liberated metal dissolves therein at the regular working temperature. I have discovered, however, that both alkali and 90 alkaline-earth metals may be obtained at a high efficiency as a result of electrolysis in the secondary cell at a convenient and economical temperature if the electrolyte consists of a metallic compound, containing 95 carbon and nitrogen, such for example as the corresponding metal cyanid or cyan-

amid, or of a stronger cyanid or cyanamid, or a mixture of such salts, and that by the use of such an electrolyte no portion of the heavy metal in the alloy can be carried along as an impurity. I thus not alone improve the product, but I further obviate the necessity for the very careful regulation of temperature, current density and composition of alloy necessitated by the use of the electrolytes heretofore proposed. In producing metallic sodium I regard pure sodium cyanid as the best secondary electrolyte; but potassium cyanid or mixed sodium and potassium cyanids may also be employed owing to the fact that potassium cyanid is a stronger compound than sodium cyanid and is not decomposed by metallic sodium. I have discovered that potassium cyanid is the most suitable cyanid for the production of the metal potassium. In the above electrolytes the corresponding cyanamid salt may be substituted for cyanid, or a mixture of such cyanamids and cyanids may be employed.

In the production of metallic lithium, calcium, barium, or strontium by this process, sodium or potassium cyanid may be employed as the electrolyte, at the beginning of the operation, but the liberated metal—lithium, calcium, barium, or strontium—will reduce the molten cyanid in whole or in part, in course of time, to the corresponding cyanamid salt, that is to say, sodium or potassium cyanamid. These molten cyanids and cyanamids constitute admirable electrolytes in connection with anodes of lead-sodium, lead-potassium, lead-barium, lead-lithium, or of any other suitable heavy metal, such, for example, as tin, combined with an alkali or alkaline-earth metal, for the reason that the heavy metals do not form corresponding salts which can exist at the temperature of the operation,—normally a moderate red heat,—the only stable cyanids or cyanamids at red heat being those of alkali or alkaline-earth metals; and further, that neither the heavy metals nor alkali or alkaline-earth metals are soluble in molten cyanid or cyanamid. The molten alkali cyanids and cyanamids, too, are especially suitable for use as electrolytes, because of their low melting points, and great fluidity, and the fact that no narrow limits of temperature are necessary, which obviates the necessity for extremely careful regulation.

The use of a cyanid is free from objection for the reason that should any molten cyanid run out into the air or should such substance escape in the form of vapor, it would immediately burn to cyanate, which is harmless; and no odor of hydrocyanic acid is apparent, for the reason that the cyanid is not used in solution and there is no hydrolysis. The cyanamids are harmless.

Other alloys, more or less suitable for the purpose in question, may be made by electrolyzing various fused salts in connection with a molten metallic cathode, among which may be mentioned alloys of each of the alkali and alkaline-earth metals with not alone 70 lead or tin, but in some cases with zinc, aluminum, etc. Hence, by the expression "heavy metals" I mean to include for the purpose of this specification, all metals not included in the alkali or alkaline-earth 75 group of metals.

It has been customary in electrolyzing molten salts of different kinds to add some fluxing agents for the purpose of lowering the melting point, increasing the fluidity, 80 bringing oxids into solution, etc. When such a mixture of salts is electrolyzed over a molten metallic cathode the voltage and current density required to economically supply all the heat required in the process, while 85 obtaining a good current efficiency, etc., are so high that all salts in the mixture are decomposed and all of the metals are liberated in contact with the surface of the alloy. Thus, in the electrolysis of molten sodium 90 chlorid over a lead cathode, as ordinarily practised, the current density is so high that any metallic chlorid or soluble salts whatsoever, whether of potassium, lithium, calcium, barium, strontium, etc., will be decomposed 95 simultaneously with the sodium chlorid and their metals will become a part of the alloy.

In the electrolysis of ordinary sodium chlorid for instance, which contains calcium sulfate as an impurity, which substance however dissolves perfectly in the molten sodium chlorid, the calcium sulfate is decomposed continuously by the current and the calcium enters the alloy together with the sodium, and if steam be afterward injected 100 into the alloy the calcium will be removed along with the sodium. The other common impurities, such as iron oxids, silica, etc., do not fuse perfectly, but settle out as 105 impurities.

In the electrolysis of molten sodium chlorid on a large scale, it is desirable to add a certain proportion of potassium chlorid to the bath for the purpose of slightly lowering the working temperature, and the process 115 may then be advantageously conducted at temperatures ranging from 800° down to 700° C., if desired. The alloy will then contain both potassium and sodium, but the presence of a small percentage of potassium 120 in metallic sodium is not found to be objectionable for the usual purposes for which sodium is required. It is of course not absolutely necessary in electrolyzing molten sodium chlorid, for instance over a lead 125 cathode, to employ any potassium chlorid whatever, but certain advantages are obtained by the use of at least 2% of this com-

pound; and this percentage may be increased up to 25%, if desired. Similarly in electrolyzing molten potassium chlorid it is desirable to add from 2 to 25% of sodium chlorid. 5 Lithium chlorid requires the addition of sodium or potassium chlorid,—not to lower its melting point, but to increase the current efficiency. If the primary bath is composed principally of molten calcium chlorid it may 10 be desirable in some cases to add 10% or more of sodium or potassium chlorid or fluorid, or one or more of the alkaline-earth chlorids or fluorids; and the same procedure may be taken in the case of barium chlorid 15 and strontium chlorid. In general, it may be stated that no hard or fast rule may be laid down to be followed concerning these mixtures of salts, and it must be borne in mind that they all will be decomposed by the 20 current if the voltage and current density be sufficiently high.

The molten metallic cathode should be a body of metal large enough to act as a storage reservoir for the alkali or alkaline-earth 25 metal, as well as for heat; and it may ordinarily contain from 5% to 25% by weight of the light metal. It should be kept in constant circulation and this circulation should not be too sluggish in order to preserve an 30 effective balance between the respective cells. This makes it possible to run either half of the furnace for several hours, while the other half is short circuited; and especially does it tend to equalize the temperature 35 throughout the whole apparatus. This is particularly true when the apparatus is compact and well inclosed in non-conducting brick work, or other heat insulating material, resulting in a conservation of the 40 energy required throughout the process. It may be here noted that the provision of an electrolyte comprising a suitable metal cyanid or cyanamid, permits of this particularly desirable feature since it allows the 45 secondary cell to be operated at the same or substantially the same temperature as the primary. The principal source of electrical heat should be in the primary bath and the voltage and current density should there be 50 relatively high. If the temperature of the primary bath is 750° C., the temperature of the circulating alloy throughout the furnace will be approximately 750° C., and the temperature of this moving body of metal will 55 determine to a large extent the temperature of the operation in the secondary furnace, which will ordinarily be but very slightly lower than that of the moving metal; but the temperature of the secondary 60 electrolyte may be, in fact, maintained as much as 100° C. lower than that in the primary, if desired, by employing a very low current density in the secondary, by exposing the iron cover to heat radiation in the

air, by conducting some of the heat away 65 through an extra heavy cathode with outside copper connections, etc. Here again the use of alkali cyanids and cyanamids is beneficial owing to their low melting points, which, of course permits the electrolyte to 70 remain fluid over a large range of temperature.

Other advantages arising from the use of my process will be hereinafter set forth and more particularly pointed out in the appended claims.

In the accompanying drawings, which illustrate one form of apparatus adapted to carry out my process: Figure 1 is a vertical section of a double compartment furnace, 80 said section being taken on the line I—I of Fig. 2. Fig. 2 is a horizontal section of said furnace taken on the line II—II of Fig. 1. Fig. 3 is a transverse vertical section taken on the line III—III of Fig. 2. Fig. 4 is a 85 fragmentary section taken on the line IV—IV of Fig. 3.

The furnace casting or inner container 1 should preferably be made of cast iron or cast steel, and the inner walls of each compartment should preferably be lined with refractory material 2, such as alumina or magnesia. The furnace casting is inclosed at the bottom and on all sides by heat insulating material 3, preferably brick or the like. The furnace comprises two principal compartments, a primary compartment 4 and a secondary compartment 5, these compartments being separated by a septum or wall 6 which preferably forms an integral 95 part of the casting 1. In vertical section, this wall has been shown in the form of an inverted T; the bottom flanges 7 thereof serving to support the adjacent side linings 2. The primary anodes 8 extend through 100 the top of the primary compartment and are preferably made of some form of carbon; graphite being particularly well adapted for the purpose. This primary compartment is covered with a slab 9 of suitable refractory material not affected by chlorine or other corrosive gas which may be liberated at the anodes. The gases so liberated are conducted away through the flues or vents 10. The secondary compartment 5 is fitted 115 with an overflow spout 11 for the purpose of conducting off metallic sodium for example, if that be the ultimate material desired; and this compartment is preferably fitted with an iron cover 12 insulated from 120 the inner container by means of an asbestos or fire-cement gasket or ring. A cast iron or other metal piston-shaped cathode 13 projects through the cover into the electrolyte 14 of the secondary cell and constitutes 125 the negative terminal of the furnace; the primary anodes 8, which constitute the positive terminal extending into the pri-

mary electrolyte 15. The body of heavy metal or alloy 16, is disposed in the bottom of the respective compartments and a plurality of conduits are provided which are 5 also filled by said alloy, such conduits affording means for effectively circulating the heavy metal or alloy, through the respective compartments. In the form of furnace illustrated, one of such conduits is 10 shown in section in Fig. 1, and has been designated 17; a passage 18 leading down into it from compartment 4 and a corresponding passage 19, leading from it to compartment 5. As will be observed from an inspection 15 of Fig. 2, these passages 18 and 19 are relatively elongated and in substantial alignment, but have their remote ends somewhat enlarged in order to equalize the flow of alloy through the chambers.

20 The second conduit 20 is in communication with the further sides of the respective compartments through passages 21 and 22, such passages also having the form of elongated slots and the conduit 20 leading therefrom to a suitable pump 23. This pump is 25 preferably of the centrifugal type, but any suitable apparatus may be employed for this purpose which is adapted to efficiently circulate the mass of alloy. The movement of 30 the mass of fluid alloy through the compartments results in stirring up the respective electrolyte bodies, since such bodies float upon the surface of the alloy in the respective compartments. The circulation of 35 the alloy may be effected either intermittently or continuously by mechanical means or otherwise, and suitable means, such as a hopper 24, may be provided for permitting the continuous or intermittent introduction 40 of the salt required in the primary compartment.

For the production of metallic sodium, I 45 prefer to employ fused sodium chlorid, or a mixture thereof with other compounds, as the electrolyte 15, while the electrolyte 14 should be a cyanogen compound. The heavy 50 molten metal, such for instance as lead-sodium alloy, extends up into and covers the bottom of each compartment and thereby serves to separate the respective electrolytes 55 by efficiently sealing the channels or conduits connecting the primary and secondary cells.

The process may be carried out either in 60 intermittently or continuously in the double compartment furnace described; or the two compartments or cells may be entirely distinct and separate from each other;—that is, the alloy may be made in one furnace and afterward transferred bodily to a separate furnace and there decomposed, such procedure being obviously within the scope of the invention.

In operation, should it be decided to man-

ufacture simply sodium, so that such material may be accumulated, sodium chlorid, for example, would be introduced through the hopper 24 and electrolyzed by suitable current, chlorin being evolved and passing off through the vent 10 while the sodium 65 combines with the lead or other heavy metal which forms the cathode in the primary cell, to form the lead-sodium alloy. This alloy in turn becomes the anode of the secondary cell, molecules of the sodium-cyanid there- 70 in being momentarily dissociated, the released sodium being deposited upon the cathode while the cyanogen anions combine with fresh sodium from the surface of the alloy, the accumulated sodium upon the 75 cathode rising to the surface of the electrolyte at 25 from whence it may be drawn off continuously or intermittently; and the electrolyte hence remaining substantially unconsumed. This action is the same with 80 all of the alkali metals, such for example as sodium, potassium, lithium, etc., the resultant product being delivered through the overflow spout 11.

The closures 9 and 12 are preferably cov- 85 ered with a layer of suitable material to form a seal and further to aid in retaining the heat. I prefer to use common salt (NaCl) for this purpose when using sodium chlorid as an electrolyte in the primary cell. 90

In conclusion I particularly wish also to call attention to the low melting points of the cyanids, which are considerably below the temperature required for the formation of the alloy. These compounds, too, being 100 free from water or water-forming constituents and also being non-halogen compounds are not subject to the objection hereinbefore referred to, to wit, a liability to attack the heavy metal of the alloy, to form soluble 105 compounds therewith at the temperature of the operation, which temperature as aforesaid approximates a red-heat.

What I claim, is:

1. The process of producing metal which 110 comprises electrolyzing a fused compound containing carbon, nitrogen and the métal to be produced, by passing a current of electricity therethrough from a body of material containing the desired metal and an- 115 other metal.

2. The process of obtaining a metal which comprises electrolyzing a salt containing the desired metal in combination with a carbon and nitrogen radical, with an anode com- 120 prising a body of alloy containing the desired metal and another metal incapable of forming a combination with a carbon and nitrogen radical at the temperature of the operation.

3. The process of obtaining a metal which comprises passing a current of electricity through a molten mass containing the de- 125

sired metal in combination with a nitrogen and carbon radical, from an anode consisting of a body of molten alloy containing the desired metal and another metal which 5 is incapable of forming a combination with a carbon and nitrogen radical which is stable at the temperature of the operation.

4. The process of producing alkali metal which comprises electrolyzing a fused cy- 10 anogen compound of said alkali metal, by passing current from a fused alloy comprising said alkali metal and another metal.

5. The process of producing alkali metal which comprises electrolyzing a fused cy- 15 anogen compound of said alkali metal, by passing current from a fused alloy comprising said alkali metal and another metal which does not form a stable cyanid at the temperature of the molten alloy.

20 6. The process of obtaining a metal which comprises electrolyzing a fluid mass containing a cyanogen compound, by passing an electric current through said mass from an anode comprising a body of alloy containing the desired metal and another metal which does not form a stable cyanogen compound at the temperature of the operation.

7. The process of obtaining a metal which comprises electrolyzing a fluid mass containing a cyanid, by passing an electric current through said mass from an anode comprising a body of alloy containing the desired metal and another metal which does not form a stable cyanid at the temperature 35 of the operation.

8. The process of obtaining a light metal belonging to the group of metals which form stable cyanids when molten, which comprises passing an electric current 40 through a molten bath containing one or more stable cyanogen compounds non-decomposable by the desired metal, from an anode consisting of a molten alloy containing a heavy metal and the desired light 45 metal.

9. The process of obtaining a light metal belonging to the group of metals which form stable cyanids when molten, which comprises passing an electric current 50 through a molten bath containing one or more stable cyanids non-decomposable by the desired metal, from an anode consisting of a molten alloy containing a heavy metal and the desired light metal.

55 10. The process of obtaining a light metal belonging to the group of metals which form both stable cyanids and chlorids when molten, which consists in electrolyzing a fused chlorid of the light metal in a primary 60 electrolytic cell over a cathode which forms a fusible alloy with said metal, and thereafter using said alloy as an anode in a secondary electrolytic cell containing an electrolyte comprising a molten cyanid of the light metal of the electrolyte.

light metal, depositing the light metal at 65 the cathode.

11. The process of obtaining an alkali metal which comprises electrolyzing a mass of alkali metal cyanid, by passing current therethrough from an alkali-metal-alloy 70 anode, dissolving the alkali metal out of said alloy and depositing said alkali metal at the cathode without consuming the electrolyte.

12. The process of obtaining an alkali 75 metal which comprises electrolyzing a primary electrolyte containing a fused chlorid over a cathode which forms a fusible alloy with the alkali metal, thereafter dissolving said alkali metal out of said alloy by electrolyzing a secondary electrolyte containing an alkali metal cyanid while using the alkali metal alloy as an anode therein, the alkali metal depositing at the cathode without consuming said secondary electrolyte. 80

13. The process of producing sodium which comprises electrolyzing a fused cyanogen compound of sodium by passing current from a fused alloy comprising sodium and another metal. 85

14. The process of obtaining sodium which comprises electrolyzing a fluid mass containing a cyanid by passing an electric current through said mass from an anode comprising a body of alloy containing the desired 95 metal and another metal which does not form a stable cyanid at the temperature of operation. 90

15. The process of obtaining a metal belonging to either the alkali or alkaline earth 100 groups which comprises electrolyzing a fluid mass of the desired metal belonging to said groups in a primary electrolytic cell over a cathode which forms a fusible alloy with said metal and thereafter using said 105 alloy as an anode in a secondary electrolytic cell containing an electrolyte comprising a molten cyanid of the light metal thereby depositing the light metal at the cathode.

16. The process of obtaining sodium which 110 consists in electrolyzing fused sodium chlorid in an electrolytic cell over a cathode which forms a fusible alloy with said sodium and thereafter using said alloy as an anode in a secondary electrolytic cell containing an electrolyte comprising a molten sodium cyanid, depositing the sodium at the cathode. 115

17. The process of obtaining an alkali or alkaline earth metal which comprises electrolyzing a mass of the metal cyanid containing the desired alkali or alkaline earth metal by passing a current therethrough from an alkali or alkaline earth metal alloy, dissolving the alkali or alkaline earth metal 125 out of said alloy and depositing said metal at the cathode without consuming the electrolyte. 120

18. The process of obtaining sodium which comprises electrolyzing a primary electrolyte containing fused sodium chlorid over a cathode which forms a fusible alloy with 5 said sodium thereafter dissolving said sodium out of the alloy by electrolyzing a secondary electrolyte containing sodium cyanid while using the sodium alloy as an anode therein, the sodium depositing at the

cathode without consuming said secondary electrolyte.

In witness whereof, I subscribe my signature in the presence of two witnesses.

CHARLES E. ACKER.

Witnesses:

WALDO M. CHAPIN,  
JAMES DE ANTONIO.